

## UNITED STATES PATENT OFFICE.

THEODOR HELLTHALER, OF GRANSCHUTZ, GERMANY, ASSIGNOR TO THE FIRM: HUGO STINNES RIEBECK MONTAN UND ÖLWERKE AKT. GES., OF HALLE-ON-THE-SAALE, GERMANY.

## PROCESS OF REFINING MINERAL OILS.

No Drawing. Application filed August 1, 1925, Serial No. 47,608, and in Germany December 3, 1924.

This invention relates to the process of refining mineral oils of every description. This process was hitherto generally carried out by treating the oils with sulphuric acid whereby the basic substances, and such which cause the formation of resins and asphalt are removed, but at the same time a number of undesired secondary reactions take place, which for a long time have been the object of particular investigations. For instance, it is well known, that, besides acid resins, numerous oxidation products and sulfo compounds are formed, which, owing to their generally rather viscous consistency contain considerable quantities of refined products. Furthermore by the subsequent inevitable washing process the oils are emulsified, thereby causing the loss of considerable quantities of oil.

Many experiments have been made to substitute other chemical agents for sulphuric acid. Thus among other substances anhydrous tin tetrachloride has been proposed as a refining agent. However, on subjecting mineral oils to the action of this product under the conditions described in the literature a more or less violent reaction with the production of heat is observed which depends upon the quantity of the unsaturated compounds present. Each added drop is at once enclosed in a dark, spongy resinous mass, whereby the refining agent is prevented from further action upon the mineral oil. Therefore with this method a sufficiently refined and clarified oil can only be obtained when employing considerable quantities of refining agents, and with very great loss of oil.

Now I have found that these disadvantages are avoided by subjecting the mineral oils to tin tetrahalogenids in a finely distributed or diluted form. This may be effected by the adsorption of the tin compounds by suitable solid finely distributed bodies such as fuller's earth, silicate of alumina, infusorial earth (kieselguhr), clay, activated carbon, soda ash, calcium carbonate and the like. Instead of solid diluents, liquid organic solvents not participating in the reaction may also be employed, such as chlorinated hydrocarbons, petroleum ether, benzine and the like.

When tin tetrahalogenids, for instance tin tetrachloride  $\text{SnCl}_4$ , in this form is made to act on mineral oils, the violent reaction be-

tween the reagent and the oil is moderated. Moreover, owing to the dissemination of the refining agent upon a greater surface by far fewer quantities of the reagent will suffice, the resinous or asphaltic masses simultaneously produced being adsorbed by the solid substrata or dissolved by the organic solvents. Furthermore, the employing of solid substrata has the advantage of manipulating such powdery substances more conveniently than the violently fuming and corrosive tin tetrahalogenid. Of course solid and liquid diluents may be used simultaneously.

With my improved method a subsequent distillation is not needed in most cases, but refined products of light color and free from asphalt are immediately obtained. It is advisable to follow up the treatment of the oils by a subsequent treatment with suitable basic substances such as bleaching earth or the like, whereby at the same time the hydrochloric or other acid formed is neutralized, and the oils are further clarified. The tin employed may be easily recovered from the residue by known methods.

The process forming the object of the present invention may be employed for refining mineral oils of every description, such as petroleum or petroleum distillates, shale oil, or shale oil distillates, lignite tar primary or low temperature distillation, tar or its distillates and the like.

## Examples.

(1) A dark, opaque dynamo oil showing specific gravity 0.906, viscosity at 20° C. 11.5 (Engler's scale), asphalt 0.1 p. ct., was treated under violent stirring with 6 p. ct. by weight of a mixture consisting of 1 part of tin tetrachloride and 2 parts of earth, filtered and shaken with 5 p. ct. of alkaline bleaching earth or water. A bright yellow, neutral lubricant was obtained having the following properties: specific gravity 0.901, viscosity at 20° C. 10.6 E., asphalt none.

(2) An asphalt-like lubricating oil not well adapted for being refined obtained from Mexican raw oil showing specific gravity at 20° C. 0.948, viscosity at 50° C. 9.1 E., asphalt 0.2 p. ct., was treated with 12 p. ct. of its weight of a powder consisting of equal parts of tin tetrachloride and aluminum silicate, and a refined product wholly free from asphalt and having the following properties

was obtained: specific gravity at 20° C. 0.938, viscosity at 50° C. 8.5 E, asphalt none.

The oil was of a yellow color and had a better smell than the original product.

6 1 claim:

1. The process of refining mineral oils consisting in treating the oils with tin tetrahalogenids precipitated upon solid, finely distributed carriers.

10 2. The process of refining mineral oils con-

sisting in treating the oils with finely distributed tin tetrahalogenids and thereafter with basic bleaching earth.

3. The process of refining mineral oils consisting in treating the oils with tin tetrahalogenids finely distributed in an inert diluent and thereafter with basic bleaching earth.

In testimony whereof I affix my signature.

THEODOR HELLHALER.